

June 7, 1927.

1,631,171

H. F. WEISS

UTILIZING WOOD WASTE

Original Filed May 19, 1921



Inventor

Howard F. Weiss  
By his Attorneys  
Fannie Davis Morris & Edmunds

Patented June 7, 1927.

1,631,171

# UNITED STATES PATENT OFFICE.

HOWARD F. WEISS, OF MADISON, WISCONSIN, ASSIGNOR, BY MESNE ASSIGNMENTS, TO  
WOOD CONVERSION COMPANY, OF CLOQUET, MINNESOTA, A CORPORATION OF DELA-  
WARE.

## UTILIZING WOOD WASTE.

Application filed May 19, 1921, Serial No. 470,967. Renewed April 19, 1927.

There are now on the market three general types of wall board made from wood. The first type is made as follows: Round wood is ground into a mechanical pulp on grinding equipment such as is used in making ordinary ground wood pulp for paper manufacture. To this ground wood pulp is added a certain amount of chemical pulp to give added strength to the finished product, then the mixture is flowed over an ordinary board machine into a sheet of paper having the thickness of ordinary card-board. At the end of the paper making machine the sheets are wound into rolls of a size convenient for transportation. The wall board is made from them by unrolling five rolls or more simultaneously and gluing or cementing the various sheets of paper together, usually with an adhesive such as sodium silicate. The sheets of paper or card-board thus glued together are then cut to the desired size and dried and in this form are commercial wall board. Some manufacturers use waste papers in whole or in part instead of ground round wood, but without change in the essentials of the process as above outlined. Walls boards of this type are sold in the United States in greater tonnage than those of any other type.

A second type of wall board now on the market is made by grinding the wood to a pulp and then beating the pulp in standard paper making beaters and finally flowing it into trays; these trays are then put into a hydraulic press and the mass is compressed into a dense product which is then removed from the press, dried, trimmed, and surfaced. Chemical pulp can be substituted in whole or in part for ground wood pulp in this type of board. This board consists of but one layer, and usually is denser and has a more compact surface than wall board made from paper sheets.

A third type of wall board is made by gluing or cementing between two heavy sheets of paper, slats of wood placed side by side. This board is expensive because of the cost of the wood slats and because of the relatively large quantity of sodium silicate or other adhesive that must be used in holding the slats together and in fastening the covering sheets firmly to the wood. The covering sheets are relatively tough and thick and have the characteristic appearance and surface texture of paper.

These three types include all of the various varieties of wood wall board now on the market in a large way. They all involve the step of first preparing a wood pulp either mechanically or chemically in standard pulp making equipment. Such equipment is, from its very character, expensive to install and expensive to operate, and requires large floor area, particularly for the driers of the paper making machine. Furthermore, the manufacture of all of these types starts with logs of good size and quality, which, if not used in the manufacture of wall board, could well be used in the manufacture of newsprint paper and even more expensive papers. And aside from the standard pulp-making equipment used in these processes, the boards themselves are made on large and expensive machines requiring large floor area; the single exception being the one ply board made on a press as above outlined.

All of the wall boards above described rely mainly for their strength upon the interlacing and interlocking of the fibers and, therefore, their processes of manufacture aim to make a pulp having fibers as long as possible. In general, for best results, this requires the use of round wood of good quality and of grinding equipment well designed and carefully maintained. But around every saw mill there accumulates large quantities of what may be termed saw mill offal or wood waste, such as slabs, edgings, trimmings, sawdust, shavings, and bark. Some of this material such as the slabs and edgings, is marketable, under favorable shipping conditions, to paper mills, but though the quality of fiber in the slabs and edgings is as good or better than the general run of fiber from round wood, the pieces of wood are in such physical condition that they are not readily reduced to a pulp, with the result that the yield of fiber is low, the quality of the pulp is poor, and the practical difficulties of operation are enormous.

Any wall board process that depends for its raw material on grinding round wood on a stone requires the expenditure of large quantities of power. For example, a ton of ground wood pulp, suitable for making the plies of a wall board, requires 1200 to 2400 horsepower hours for grinding alone. This great quantity of power is consumed, partly in the mechanical work of tearing the fibers

one from another, but more largely in frictional loss at the surface of the stone where it rubs with heavy pressure on the log of wood and where the log acts as a brake on the stone. This frictional loss is dissipated in the form of heat and the heat is carried away in the cooling water and thus is lost. The cooling water, after separation of the fibers, is ordinarily run to waste.

10 It is an object of the present invention to produce a wall board consisting essentially of a single ply, this board being free from sodium silicate, and being uniform throughout. The board may have a surface that is 15 dense and capable of taking a good finish and even a high polish, and if desired, can be ornamented by graining and painting methods now well developed in the decoration of sheet material, such for instance as 20 sheet metal.

It is a further object of the present invention to produce a wall board of acceptable character from saw mill offal such as 25 slabs, trimmings, edgings, sawdust, shavings, and even bark and to do this with a power consumption far below that ordinarily needed and in machinery and buildings less expensive than those now needed for the production of wall board from 30 ground wood or from chemical pulp. Other objects and advantages of the present invention will become clear from the following description which is to be taken in conjunction with the accompanying drawings, 35 wherein:

Figure 1 is a diagrammatic representation, in elevation, of a complete plant for making wall board by the present process, and Fig. 2 is a diagrammatic plan view of 40 the same.

The wall board of the present invention comprises a binder and a filler and the novelty in the product lies particularly in the binder and in its combination with a filler 45 of special character. There is also novelty in the process of making and using the binder, particularly for the manufacture of a wall board such as that hereinafter described.

50 The binder consists essentially of lignocellulose gelatinized by mechanical disintegration preferably in the presence of water and without the use of any gelatinizing chemical. This binder, when dry, is a hard, 55 horny mass having good binding qualities, and yet offering no impediment to usual woodworking operations, such as sawing, planing, chiseling, and the like. The binder is preferably made from sawdust or somewhat larger particles of raw wood as by 60 crushing or rolling the wood particles between relatively rotating discs whereby the fibers are torn apart and subjected to pressure in the presence of water, and ultimately 65 are converted substantially entirely into a

gelatinized mass. If wood particles other than sawdust are used as the raw material for the binder, they are preferably obtained by chipping, hogging or shredding mill waste or offal, and not by grinding solid 70 wood on a stone as in pulp making. These chips or particles advantageously can be water-logged to facilitate their mechanical disintegration and their conversion into gelatinous material.

75 The filler need not be separate fibers, as excellent results are had by using bundles of fibers such as sawdust, preferably screened to take out the finest and the coarsest particles. Incompletely gelatinized wood particles can constitute the filler, and it is possible to use ground wood pulp or cooked wood pulp or old newspapers beaten to a pulp as the filler, but as hereinafter pointed out at length, there are many practical advantages in using sawdust or equivalent unground and unbeaten fibers grouped together or aggregated as in the living tree.

80 The details of the process and of the product in their preferred embodiments will be 85 better understood from the following disclosure.

#### *The binder.*

Starting with saw mill offal or waste, 95 such as slabs, edgings, trimmings, shavings, and even bark or with mixtures of these, or starting with paper mill offal or waste such as crooked bolts, or limbs or branches such as are commonly left in the forest, either 100 with or without preliminary removal of the bark by usual methods, as in the so-called drum barker, I pass the waste through a "hog" such as is used at saw mills for cutting up waste wood to make it suitable for 105 fuel, or through a "chipper", such as is used in preparing wood for the soda, sulfite or sulfate process, or through a "coarse shredder", such as is sometimes used at saw mills 110 in place of a hog to reduce wood to small chips or fragments. If desired, a hog and the shredder may be used in conjunction, the hog cutting the wood into fragments say two inches long, and the shredder beating these fragments into smaller pieces. Good 115 sound round wood can of course be used as raw material but mill waste is much cheaper and is entirely satisfactory. All of these operations which, for lack of a better name, I will hereinafter designate as "chipping", 120 are carried out by a cutting action which requires very much less power than if the waste were reduced to a pulp by holding solid blocks of it against a rapidly rotating stone as in grinding wood for ground wood pulp. Also, the product resulting from chipping is entirely different from ground wood pulp.

125 Thus, by chipping, the saw mill or paper mill offal is reduced to a mass of chips or 130

wood particles of a size about one-half inch in length by one-eighth inch in diameter, or less. This material is then passed over a series of screens and the very fine particles, 5 which for want of a better name I will hereinafter designate as "fiber aggregates", are collected and stored in a bin. These fiber aggregates may be as fine as ordinary sawdust and in fact by starting with sawdust, 10 such as is obtainable at any saw mill I can dispense with the chipping procedure described above, for the material is already fine enough to be called "fiber aggregates" and to be used as such. In the drawing, the 15 bin for holding the sawdust of other fiber aggregates is marked with reference character 1.

The next coarser grade from the screens, which I prefer to call "small wood particles", 20 goes ultimately to a storage bin 2, and the coarsest particles are returned from the screen to the shredder for retreatment and ultimate conversion into "small wood particles" and into the smaller "fiber aggregates". If the saw mill waste is all in the 25 form of sawdust, or other like small particles, the chipping and shredding steps can be omitted for the material that is to go into bin 2, the same as for that supplied to bin 1.

30 The small wood particles that are to be supplied to bin 2 can with advantage be given a water-logging treatment after being taken from the screen and before being delivered into the bin. If sawdust is to be 35 used as a raw material, the procedure is the same. This water-logging is used because wood that is wet is very much weaker and can be torn apart with less expenditure of energy than wood that is dry—the fibers 40 separate from one another more easily. For example, wet wood has, in compression, about one-half to one-third of the strength of dry wood. This water-logging can be 45 done conveniently by first submerging the small wood particles in water heated near or preferably to the boiling point, and then, while the wood particles are submerged in a closed tank, subjecting the mass to pressure such as steam pressure to force the hot water 50 into the fiber aggregates.

As an alternative procedure, the small wood particles can be thoroughly heated in the hot water and then, while the temperature of the water is near or at the boiling 55 point, cold water can be added to cause contraction of the expanded air and gases of the wood particles, thereby drawing water into the pores or voids of the particles.

60 As another procedure, the small wood particles while hot from the exposure to hot water, can be dumped into cold water to cause contraction of the expanded air and gases as above described. Under some circumstances, it is more economical merely to 65 let the hot water and the submerged wood

particles cool by radiation, for by so doing large quantities of water will be drawn into the pores and voids of the wood.

By such a treatment, small wood particles (and sawdust) can be so thoroughly saturated with water that they will sink in water in an hour or less. If they were merely submerged in water it would take months and, in the case of resistant woods, years, before the wood soaked up enough water to sink. 70 The heating in hot water is not intended to be a cooking operation and there need be no chemical present to effect cooking. Nevertheless, the hot water dissolves out some or perhaps all of the highly soluble constituents 75 of the wood. When western larch is used as the wood, this is a valuable feature of the process, because of the possibility of recovering valuable sugar-making ingredients from the liquor. 80

85 The small wood particles (which, as above explained, may be nothing more than sawdust or may be larger particles), now thoroughly saturated with water and consequently in a very weak condition, are passed 90 into hopper 2 (Fig. 1) preparatory to delivery into a machine 3 whereby they are torn apart and reduced to separated fibers. Since wood is weaker hot than cold, I prefer 95 to pass the small wood particles into this machine while they are still hot from the water-logging procedure. If the chilling with cold water has completely cooled the wood particles, it is sometimes advisable to again heat them up before delivery into machine 3. The machine 3, for separating the 100 fibers, may be constructed in many ways, but best results have been obtained by me in an apparatus having two large discs of metal, one of which is rotatable with respect to the other, and between which the hot and water-logged wood is subjected to a rolling action 105 to tear, or more strictly speaking, crush the fibers one from another. Good results have been obtained by use of disc grinders commonly known as "corn crackers", of which the 36 inch single disc mill of Bauer Bros. Co., Springfield, Ohio, U. S. A., is a good illustration. The details of such a disc grinder or corn cracker are well illustrated 110 in U. S. Letters Patent Nos. 565,690, issued August 11, 1896, 817,610, issued April 10, 1906. 115

120 In such a machine, the action of tearing the wood fibers apart resembles somewhat the disintegrating effect of rolling a match under foot on the floor, excepting, however, that because of the relative rotative movement of the discs, each piece of wood or bundle of fibers has a gyroscopic motion about the axis of the rotating disc so that not only are the fibers and bundles of fibers 125 subjected to a crushing action, but they are subjected to a twisting effect. As one disc rotates with respect to the other, the small 130

wood particles or bundles of fibers will naturally take up positions along radii of the rotating disc, and since their outer ends travel through a greater distance than their inner ends, there will be a decided tendency for the fibers to slip longitudinally with a twisting movement. That is to say, there is not only a crushing pressure perpendicular to the axes of the individual fibers, but there is a strain, in shear, superimposed on the crushing strain and parallel to the axes of the fibers, or more strictly speaking, radial to the rotating plate of the machine. It will be understood that the two plates of the machine between which the particles are rolled have slightly concaved faces and can be roughened or surfaced to accelerate the disintegrating action or fiber liberation. Both plates may rotate in opposite directions, or one may be stationary and the other rotatable. The working faces of the discs are preferably of metal; but of whatever material, the surfaces are adjusted in such manner that they do not touch. It is also important that means be provided for adjusting the distances between the plates in accordance with the size, character and origin of the wood particles under treatment, and the character of the product desired. It is a rolling and twisting action rather than a grinding action that gives best results in the manufacture of the products hereinafter described. Too much of the grinding action produces too large a percentage of wood flour, as distinguished from fiber pulp.

The power consumed for reducing wood to pulp by first chipping, then shredding and then rolling the small wood particles between two relatively moving discs as above described, is much less than that required for tearing the fibers apart on an ordinary paper mill grindstone; for not only has the chipping and shredding cut the fibers from the solid wood, but the resistance or strength of the particles has been reduced by water-logging and by heating, and, furthermore, the disintegrating or fiber-liberating power is applied to the particles in compression and in shear, and therefore along their lines of least resistance. Also, in this process, friction and frictional losses have been reduced to a minimum. The bundles of fibers act as rollers between the moving surfaces while rolling one upon the other. If desired, water may be passed through the mill with the particles, but this is to facilitate the flow or flushing out of the material and not because of the cooling action of the water. In fact hot water can best be used for this purpose because of its effect in lowering the resistance of the wood to crushing action and similar disintegrating stresses. When water is used, or even without the water, it is well not to rotate the mill too fast, for not only is there a power loss due to the inertia

of the water and the material being ground, but also there is apt to be a bad effect on the product because of too great breakage of individual fibers and too high a production of wood flour. The material delivered from machine 3 can be screened and the wood particles of proper size to be called fiber aggregates can be separated out and delivered to bin 1 as a substitute for, or an admixture to, the sawdust therein.

To reduce the wood to individual fibers, it may be passed repeatedly through the same fiber liberating machine, screens being used to separate out those fibers that have been sufficiently reduced and returning to the machine for further treatment only the coarser bundles or shives. Or, if desired, a series of fiber liberating machines may be used, in each succeeding one of which the relatively moving surfaces are so adjusted as to give best disintegrating action on the partially reduced wood with which it is supplied. The latter procedure is preferable.

Such an arrangement is indicated diagrammatically in Fig. 2 of the drawings, where the material delivered from disc grinder 3 is carried by an elevator 4 to a hopper 5 adapted to deliver to a disc grinder 6. When delivered from the latter to tank 7, the mass can be lifted by pump 8 and delivered through pipes 9 or 10 to grinders 11 or 12, which, in turn, deliver to tank 13 from which the mass can similarly be pumped to other disc grinders of the series. As the wood proceeds through the series of grinders, the particles are torn apart into separate individual fibers and furthermore these fibers undergo a chemical change and ultimately are delivered from the last grinder of the series into storage tank 14 as a gelatinous, structureless mass free from chemicals of any sort and well adapted for use as a binder in the wall board of my present invention.

It is well recognized in the literature that the hydration qualities of lignocellulose or wood are not very great, and that mechanical wood pulp suffers little alteration by beating in a paper-maker's beater. But I have found that when lignocellulose or wood is crushed or rolled under pressure in a corn cracker, hydration will begin even in the first mill of the series, and the hydration will progressively increase as the wood is reduced to fiber and the fibers are broken and crumbled under pressure. The water-logging treatment to which the wood has been subjected facilitates hydration. Furthermore, the wood hydrates and approaches gelatinization more easily while it is warm or hot. However, it is entirely possible to produce gelatinized lignocellulose without giving it the water-logging treatment and by rolling and breaking the fibers in cold water instead of hot.

While the hydration or gelatinizing effect may not be very great in grinder 3 (Fig. 2), the other, and particularly the last grinders of the series, in which the plates are set close

5 together, so completely comb out, crush and gelatinize the wood fibers, that their fibrous structure disappears entirely.

The resultant product is a slimy gelatinous mass of lignocellulose. This might perhaps be called "hydrated lignocellulose", though I know of no method for determining how many water molecules have attached 10 themselves to the cellulose molecule or if indeed any such water molecules have been 15 added. I know that the chemical structure must be different from that of lignocellulose, and as appears below, the physical structure is likewise radically different. Therefore, for lack of a better name, I have herein designated 20 this material, which is to be the binder or binding element of the wall board, as "gelatinized lignocellulose". Gelatinized lignocellulose, as the term is herein used, means wood fibers (lignocellulose) that have 25 been so treated mechanically as to be completely torn and broken so that their length is but a fractional part of their original length, say for instance, one-tenth or less; furthermore, the original wood cellulose has 30 been changed chemically, though only by mechanical treatment in the presence of water, and perhaps to the extent of adding to it an unknown number of water molecules. The material, when wet, is a slime which on 35 drying shrinks enormously and is inclined to warp and forms a dense hard bone-like mass of considerable strength and without appreciable fibrous structure but inclined to split or flake, and of a color usually somewhat darker than that of the wood from 40 which it was made. Made from pine, spruce, or hemlock, the material is cream colored, and made from fir, tamarack or larch, it is somewhat darker in color. It can be made 45 readily from any of these woods, and others, but with cedar the problem is more difficult because of difficulties in chemically changing the water-resistant fibers of such a gymnosperm. To gelatinize water-resistant fibers, such as cedar, I find it expedient to 50 supply the grinders, not with water, but with an aqueous solution of sodium silicate. This is not so cheap as water alone and yields a final product that may not be entirely free from chemical additions, and therefore more likely to change in color, or otherwise, while in use as on the wall of a 55 building.

When properly made, the gelatinized lignocellulose contains no spindle shaped fibers of their original length, nor bundles of cut fibers, such as is found in "wood flour". Both physically and chemically, gelatinized lignocellulose is readily distinguishable from wood flour, though according to my experi-

ments, wood flour often results from prolonged mechanical treatments of wood fiber, as for instance, when the fiber is passed repeatedly through a Jordan.

This gelatinized lignocellulose is one of 70 the materials used by me in the production of wall board, and not only constitutes an appreciable percentage of the total material used, but acts as a binder to unite with and hold in place the other and more inert material or materials hereinafter designated as the filler.

A feature which readily may be incorporated in the above described process of making gelatinized lignocellulose is the recirculation of the water in some, at least, of the fiber-liberating machines which, with the soluble material in the wood, can be recovered in a manner similar to that described in my U. S. Patent No. 1,339,489, issued May 85 11, 1920. Furthermore, whenever a plurality of fiber liberating machines are used in series to progressively reduce the wood particles to pulp, and then to gelatinize the pulp, the circulation of the water to take out soluble 90 material (as from western larch), can be on the counter-current principle, that is to say, the water used in the last machine or grinder of the series can be filtered off from the pulpy material delivered therefrom and 95 can be introduced as the flushing water of the machine next preceding, and so on throughout the series, the strongest solution of soluble constituents being drawn off from the partially disintegrated shredded wood particles of the machine into which these particles initially were delivered.

#### *The filler.*

Stored in bin 1 is the filler for the board. 105 As above explained, this material may be sawdust or may be the finer particles obtained by screening material from the shredder, or may have been obtained by screening the material delivered from one of the grinders. I have called these smallest wood particles "fiber aggregates", and by fiber aggregates I mean five or more wood fibers still joined together as in the living tree. 110 The fibers need not, however, be of full length, and in the case of sawdust, often are not. Shingle sawdust is very good raw material for use as a filler after the very fine and the very coarse particles have been 115 screened out. This sawdust is silvery in character, light in weight, and durable, and has the further characteristic, particularly if made from cedar, that it does not hydrate during mixing nor while in use.

Instead of using a dry filler, such as sawdust, the filler may be obtained from other sources. For instance, it may consist of a part of the output of one or more of the grinders or gelatinizers above described, or 120 of coarse particles screened from the output 130

of one or more of those gelatinizers, and may be in the wet condition in which it came from the gelatinizers. Such incompletely gelatinized lignocellulose is in fact a mixture of completely gelatinized and structureless wood with wood fibers and aggregates that have been gelatinized on the surface. Such a material blends well with the completely gelatinized and structureless binder and of course is cheap, for it can be made of saw mill offal with the expenditure of but little power.

But instead of using fiber aggregates in whole or in part, as above described, I can use a more expensive filler, such as ground wood pulp, or cooked wood pulp, or mixtures of these; or I can beat up newspapers and other paper waste in a beater and use the resultant pulp, but none of these substitute fillers is as satisfactory for my purpose as fiber aggregates, such as sawdust or the incompletely disintegrated product of one of the early grinders of the series, and none of them gives a wall board that is as easy to dry, is as free from shrinkage, has as beautiful a surface, nor is as good a sound and heat insulator, as when fiber aggregates are used as the filler of the board.

#### 30      *The mixing.*

The next step in the production of the wall board consists in mixing the gelatinized lignocellulose with the filler. The latter, as above explained, may consist wholly, or in large part, of wood fiber aggregates of the same kind of wood, and even of the same origin as that which went into the gelatinizers. Or the filler may be a different wood, as for instance, one not easily gelatinized by grinding in water such as cedar or aspen. To bring the gelatinized lignocellulose and the wood fiber aggregates into intimate contact and to insure a mass uniform throughout, I pump the slimy gelatinized lignocellulose into a mechanical mixer 15, consisting of a metal trough, set at a slight incline, and provided with a power driven stirrer, comprising a central shaft on which are mounted a series of inclined stirring blades or paddles. The fiber aggregates are fed to this from hopper 1, and water may be added to thin the mix.

The relative proportions of the several ingredients of the mixture may be varied through relatively wide limits. Up to a certain point, the larger the percentage of gelatinized lignocellulose, the stronger is the resultant board. The board should contain 25% or more by dry wood weight of the gelatinized lignocellulose and 30% or more by dry wood weight of fiber aggregates. A mixture composed of 60% gelatinized lignocellulose and 40% fiber aggregates, by dry wood weight, to which enough water has been added to make the mass flow readily,

gives a very strong, stiff and satisfactory wall board. Cedar sawdust is satisfactory as a filler, though not readily adapted to the manufacture of the binder. Spruce or pine give a stronger board than cedar.

70

#### *The sizing.*

While the gelatinized lignocellulose and the fiber aggregates are being mixed, there preferably is introduced at the upper end of the mixing apparatus, a solution of sodium resinate in water. After this has been thoroughly mixed with the mass, a water solution of alum is introduced to convert the soluble sodium resinate into an insoluble resinate, all in conformity with standard practice for sizing and water-proofing paper. This treatment sizes the fiber aggregates and makes them and the finished board highly resistant to moisture. These materials may be omitted entirely when water-proofing is not desired, without impairing the strength or other characteristics of the board excepting that of its resistance to water. Normally, the percentage of sodium resinate may be from two to eight per cent of the dry weights of the other components, depending on the kind of wood used and particularly its resinous content, and the degree of waterproofing desired in the finished product. The quantity of alum is in proportion to the sodium resinate, due allowance being made for the amount of water present, etc.

95

If a fireproof board is desired, the requisite amount of ammonium sulfate can be added to the batch while in the mixer.

100

A non-mineral coloring, such as an aniline dye, can also be added, if a colored board is desired. This is particularly advantageous when the board is to be finished in imitation of mahogany.

105

Another treatment consists in coloring the gelatinized lignocellulose one color and the filler a different shade or color. This gives a very pleasing product.

110

#### *Pressing.*

The now thoroughly mixed mass of gelatinized lignocellulose and sized fiber aggregates is next delivered to a flow box 17 (Fig. 2) like those in ordinary paper making machines and so constructed as to maintain a constant head in the box with an overflow into an underground storage tank 18 (Fig. 1). A constant stream of the pulpy mass flows out of a horizontal slot in the side of the box under a gate 19. This gate is provided with a rack and pinion 20, by which it may be raised or lowered to vary the size of the stream. As the thick mixture flows through the slot it is delivered in a uniformly thick layer on a traveling canvas belt or conveyor 21 which is mounted on cylinders 22 and 23 and is reinforced along

115

120

125

130

its upper stretch by underlying and power driven endless traveling screens 24 and 25 suitably supported on drums and rollers. This prevents sagging of the canvas belt 5 while its load of material is being delivered to and from the press. To make a board about  $\frac{3}{16}$ " thick, the thickness of this layer as it flows onto the canvas belt is approximately  $2\frac{1}{2}$  inches.

10 The width of the canvas belt corresponds with the length of the board or panel to be made, and the cellulosic mass is prevented from flowing off the sides of the belt by means of two stationary baffles 26 and 27 (Fig. 2). These baffles are adjustable laterally to accommodate various widths of cellulosic mass, to accord with changes in the length of the boards to be made. In general, a board length of sixteen feet is suitable for ordinary trade demands. Thus the cellulosic mass in a relatively thick and uniform layer sixteen feet wide and one inch thick on the canvas belt is carried forward between the stationary side barriers 26 and 25 27 and ultimately passes between the platens of a hydraulic press. The canvas belt moves forward with an intermittent movement and as soon as the proper amount of the mass is between the platens, a rectangular die 28 having inside dimensions corresponding to the size of the board to be made, is lowered into the mass until it rests on the canvas sheet. The cellulosic mass is so fluid that it readily moves aside to permit 35 this lowering of the die. Then the upper platen, which fits within the die with a substantially water tight joint, is lowered into the die and compresses the cellulosic mass, while simultaneously squeezing its excess 40 water both upward and downward through suitable slots in the platens. The platens then separate, the die lifts, and the belt moves forward until a fresh amount of material has passed between the platens, when 45 the operation just described is repeated. This entire operation is done mechanically and less time than a minute is needed to press each sheet.

In order to prevent that part of the cellulosic mass which has not been pressed from flowing onto the compressed mass after the platens have been released, there are provided a series of cross baffles or partitions 50 31, adjustably attached between two sprocket chains 32 which are driven by a power driven sprocket 33 and pass over guide wheels 34, 35 and 36 as shown. These baffles or partitions, which may be made of wood, press down into the soft watery mass before 55 it reaches the press and block it off into rectangles of approximately the size needed at the press. Because of these cross baffles 31 and the side barriers 26 and 27 there is no necessity for using trays in which to form 60 and press the boards.

By changing the distance between the cross baffles 31, the width of the board can be varied in the same way that its length can be varied by changing the distance between the side barriers 26 and 27. 70

#### Drying.

The compressed cellulosic mass is carried forward from the press on the canvas belt and when picked up from this belt by an 75 endless conveyor 37 is in the form of a damp but fairly stiff compressed sheet. Conveyor 37 is adjustable vertically in supports 38 to transfer the compressed sheet sidewise into a dry kiln 39. This kiln may be of the tunnel type heated by steam coils and provided with well known means for regulating the circulation of air, its humidity, temperature, etc., to secure most effective and uniform 80 drying action and to lessen such tendency as there may be for warpage of the boards. The dry kiln removes the water from the boards so that they emerge from the kiln, 85 dry, stiff and hard.

#### Finishing.

The boards are next run through saws and cut to desired size or shape and in that form are marketable in place of wall board made by usual processes. The boards may be 90 nailed directly to the studding of a building to serve in place of lath and plaster, and like wall board now on the market, may be sawed and similarly cut to meet the needs of the builder. But unlike wall boards of 95 more usual manufacture, they do not contain enough sodium silicate or other mineral to be harmful to the saws and other edge tools of the carpenter. On the contrary, they consist throughout of substantially 100 nothing but woody material through which a saw or chisel will work as readily as through solid wood and with no more injury to the edge of the tool. The rosin size and the ammonium sulfate, if present, are 105 110 not harmful to edge tools.

But in many respects this new product is different from wall board made from paper sheets cemented together, for, if desired, the wall board of the present invention may be 115 passed through an ordinary wood planer to finish the surface, or through a sand machine to dress its surface, or between steel rolls to give the surface either a high polish or to impress in or on the surface patterns 120 or designs or to give a finish similar to burlap or canvas. Likewise, the finished and even polished face of the board may be treated much as sheet steel is now treated to give it the appearance of grained mahogany or other woods. The surface can be painted and decorated much as can be done with solid wood, excepting that it has not the characteristic grain of wood, but on the contrary, if made with fiber aggregates, has 125 130

a uniform and pleasing mottled appearance not unlike the so-called oatmeal wall papers.

- As above indicated, the process by which this novel and valuable product is made, 5 may vary in many of its details, both as to the origin of the raw materials and as to the procedure by which those materials are treated to bring them into proper physical and chemical condition to unite under 10 pressure and kiln drying into the product described in detail above. It is of particular importance, however, that no chemical need be used in the process and that water alone, together with suitable mechanical manipulations, such as cutting, rolling, and 15 twisting, properly repeated, is sufficient to convert saw mill offal such as slabs, edgings, trimmings, sawdust, shavings, and even bark, into a readily marketable product and 20 with relatively low power consumption.
- As a permissible variation from the preferred method above described, I may proceed by chipping saw mill offal such as slabs, edgings, trimmings, shavings, or bark, 25 or paper makers' waste, such as crooked bolts, saplings, and the limbs and branches 30 ordinarily left in the forest, and then mechanically disintegrating the chipped wood by crushing, in a disc grinder in the presence 35 of water, preferably hot water, as above described, and with or without the preliminary water-logging, and stopping this mechanical disintegration before the fiber aggregates 40 are completely reduced to a structureless gelatinized mass. For instance, I can carry the wood through less than six grindings and obtain a mixture consisting 45 in part, say 60%, of completely gelatinized material and in part, say 40%, of wood fibers 50 and fiber aggregates which have been gelatinized on the surface but are of woody character at the core. The exact number of grindings requisite for the desired result depends 55 on many factors, such as the character of the wood and whether it is highly resistant to water, whether it has been water-logged before grinding, how close together the grinding plates have been set and whether hot 60 water has been used in the grinders, etc. But roughly stated, three or four water grindings as above described will yield a product approximately half of which is in a gelatinized condition, and the other half 65 of which consists of fibers and fiber aggregates with but a surface gelatinization. Such a mixture, when delivered from the grinders, can be pumped into mixer 15 and thereafter can be sized, fireproofed, and then 70 flowed out in a sheet for pressing, drying and finishing in much the same way as if sawdust or equivalent dry fiber aggregates were used as a filler with a completely gelatinized binder. This alternative procedure, 75 though permissible, is in my present

opinion not so good as that first described, and yields a product having the disadvantages that it is not so cheap, not so attractive, not so good as a heat or sound insulator (because of the relative absence of voids and air pockets), more inclined to shrink and warp on drying, not so easy to dry, and not so light in weight. Also, a board so made has a monotonous appearance quite in contrast with the beautiful 75 mottled or composite appearance resulting from the use of fiber aggregates that have not been broken up by passage through a disc grinder.

As a still further permissible variation, 80 an incompletely gelatinized mass of fiber aggregates mechanically disintegrated by grinding or crushing in the presence of water, as above described, can be used as a binder for a filler consisting essentially of 85 unground fiber aggregates such as sawdust, due care being taken to keep the proportion of binder to filler within the ranges dictated by the requirements of strength, freedom from warping, undue shrinkage and the 90 like.

Preferably, the mass as it reaches the press, should comprise at least 25% by dry weight of mechanically gelatinized lignocellulose, and preferably as much as 95 40% to 60%. Likewise, the mass should contain as much as 30% or more by dry weight of fiber aggregates and preferably as much as 60% to 40%.

The apparatus whereby the process is 100 carried out obviously may vary in details without fundamentally altering either the process or the product claimed herein. Novel features of the apparatus will be 105 claimed in a separate application.

I claim:

1. The method of making wall board which consists in mechanically disintegrating small wood fibers to form a gelatinous mass, incorporating therewith a fibrous 110 filler and then pressing and drying the mass.

2. The method of making wall board which consists in mechanically disintegrating a cellulose containing material to form a gelatinous mass, incorporating therein 115 fiber aggregates to the extent of 30% to 60% by dry weight, and then pressing and drying the mass.

3. The method of making wall board which consists in mechanically disintegrating small wood particles to form a gelatinous mass, mixing fiber aggregates therewith to the extent of about 50% by dry wood weight, and then pressing and drying, substantially as described.

4. The method of making wall board, which consists in water-logging small wood particles, crushing and rolling said particles while wet between relatively rotating discs until substantially converted into gelatinous 130

lignocellulose, mixing fiber aggregates therewith, shaping and pressing into a board, and drying and finishing the board, substantially as described.

5. The method of making wall board, which consists in water-logging small wood particles, crushing and rolling said particles in water between relatively rotating discs until converted into gelatinous lignocellulose, mixing therewith an approximately equal amount by dry weight of fiber aggregates, sizing and fireproofing the mixture, shaping and pressing into a board, and drying and finishing the board, substantially as described.

10. The method of making wall board, which consists in chipping saw mill offal, forming small wood particles therefrom, water-logging said particles, crushing and rolling said particles while wet between relatively rotating discs until converted into gelatinous lignocellulose, mixing therewith an approximately equal amount by dry weight of fiber aggregates, sizing and fireproofing the mixture, shaping and pressing the mixture into a board, and drying and finishing the board, substantially as described.

15. The method of making wall board, which consists in chipping saw mill offal, forming small wood particles therefrom, water-logging said particles, repeatedly crushing and rolling said particles in hot water between relatively rotating discs until converted into gelatinous lignocellulose, mixing therewith an approximately equal amount by dry weight of fiber aggregates, sizing and fireproofing the mixture, diluting with water, flowing into a layer, pressing the layer into a board, and drying and finishing the board, substantially as described.

20. A wall board consisting essentially of a binder and a filler, the binder being a dried gelatinous mass of mechanically disintegrated lignocellulose.

25. A wall board consisting essentially of a binder and a filler, the binder being a dried gelatinous mass of mechanically disintegrated lignocellulose and the filler being essentially fibrous.

30. A wall board consisting essentially of a binder and a filler, the binder being a dried gelatinous mass of mechanically disintegrated lignocellulose and the filler consisting essentially of fiber aggregates.

35. A wall board consisting essentially of a binder and a filler, the binder being a dried gelatinous mass of mechanically disintegrated lignocellulose, and the filler consisting of untreated sawdust.

40. A wall board consisting essentially of a binder and a filler, the binder being a dried gelatinous mass of mechanically disintegrated lignocellulose, and the filler consisting essentially of fiber aggregates, said board being sized uniformly throughout, substantially as described.

45. A wall board consisting essentially of a binder and a filler, the binder being a dried gelatinous mass of mechanically disintegrated lignocellulose, and the filler consisting essentially of fiber aggregates, said board being fireproofed uniformly throughout, substantially as described.

50. A wall board consisting essentially of a binder and a filler, the binder being a dried gelatinous mass of mechanically disintegrated lignocellulose, and the filler consisting essentially of fiber aggregates, said board being dyed, substantially as described.

55. A wall board consisting essentially of a binder and a filler, the binder being a dried gelatinous mass of mechanically disintegrated lignocellulose and the filler consisting essentially of fiber aggregates, said binder being dyed one color and said filler being of a different color.

60. A wall board consisting essentially of a binder and a filler, the binder being a dried gelatinized mass of mechanically disintegrated lignocellulose and the filler consisting essentially of fiber aggregates, said binder being dyed one shade and said filler being dyed a different shade.

65. A wall board consisting essentially of a binder and a filler, the binder being a dried gelatinized mass of mechanically disintegrated lignocellulose from saw mill offal.

70. A wall board consisting essentially of a binder and a filler, the binder being a dried gelatinized mass of mechanically disintegrated lignocellulose prepared from saw mill offal and the filler consisting essentially of fiber aggregates.

75. A wall board consisting essentially of a binder and a filler, the binder being a dried gelatinous mass of mechanically disintegrated lignocellulose from saw mill offal and the filler consisting of untreated sawdust.

80. In testimony whereof I affix my signature.  
HOWARD F. WEISS.